

## UNITED STATES PATENT OFFICE

2,238,855

## DYESTUFF COMPOSITION

Norman S. Cassel, Ridgewood, N. J., assignor to  
Interchemical Corporation, New York, N. Y., a  
corporation of Ohio

No Drawing. Application January 10, 1940,  
Serial No. 313,202

5 Claims. (Cl. 8—71)

The invention relates to the art of textile decorating, and is directed particularly to new compositions intended for textile decorating, comprising dispersions of dyestuff ingredients so designed as to remain stable in storage for extended periods of time.

The conventional method of textile printing involves the application to a textile fabric of a dyestuff, or an ingredient of a dyestuff, in water solution, by means of an intaglio cylinder. In order to get the dyestuff solution thick enough to remain in the cells of the printing cylinders, and to remain in place when applied to the fabric, water-soluble thickening agents such as British gum, starch and the like are used. More recently, wetting agents have been added to the pastes to improve their printing properties. After printing, the dyes are set by various means so that they become water-insoluble, and the fabric is washed to remove the water-soluble thickeners.

Certain difficulties are encountered with these conventional dyestuff pastes. Since the fabrics printed are rather water-absorbent, prints made with water solutions, even when made viscous with the water soluble thickeners, tend to spread out slightly from the point of application, a phenomenon known as flushing. As a result, the lines in the engraving may become somewhat blurred, and very fine lines close together may be entirely lost. When the viscosities of the pastes are adjusted so that no flushing occurs, the pastes become too thick to separate cleanly from the engravings. A compromise must always be made, so that effective separation occurs without substantial flushing; and the cylinders must be so prepared as to print most easily. Fine photogravure engravings have, as a consequence, never been used with conventional textile printing pastes, because their faithful reproduction of detail would not register on the fabric. Furthermore, the engravings used must be rather deep in order to get effective printing, and considerably more paste is used than is really necessary to produce most designs.

Another disadvantage of conventional dyestuff pastes is that a substantial quantity of dyestuff may be washed out with the thickeners. This is due partially to mechanical suspension of converted dyestuff in the film of thickener, partially to incomplete conversion of the dyestuff to the insoluble form, due to the trapping of the soluble dyestuff inside of the thickener film, and, in some cases, partially to actual dyeing of the thickener. This may represent a serious loss of dyestuff.

In my copending application, Serial Number 215,585, filed June 24, 1938, of which this is a continuation in part, I have disclosed a means whereby these disadvantages may be overcome, and successful dyestuff printing can be done with photogravure and other relatively shallow engravings, with the retention of the complete de-

tail of the photogravure cylinders, and the use of a minimum of dyestuff. As therein disclosed, this means comprises the preparation of dyestuff printing pastes by the emulsification of an aqueous solution of a dyestuff or a dyestuff component capable of producing permanent dyeings on the fabrics with a water immiscible bodying composition (preferably a solution of a film-forming substance in a solvent), the dyestuff solution being in the discontinuous phase. The resultant emulsion, of optimum consistency for printing, is applied to a fabric, as with a conventional intaglio cylinder; the dyestuff is fixed on the fabric, and the fabric is then dried, with or without washing, depending on the dyestuff employed.

As the emulsion is applied to the cloth and the emulsion breaks, the dyestuff solution penetrates into the yarns of the fabric. Since the water phase and the bodying agent are mutually repellent, the non-aqueous phase prevents undue spreading of the aqueous phase. As a result, substantially no flushing occurs, and fine printing is obtained, which preserves the fine lines of a photogravure engraving even on materials which are as difficult to print as cotton flannels.

While these emulsion pastes are unusually effective printing media, a serious difficulty with their use rises from the fact that many dyestuff ingredients, particularly of the diazo type, are unstable in the presence of water, so that color strength is lost on storage of the pastes. This necessitates making up small batches of these colors at the print plant, as they are needed, with the inconvenience of measuring out small quantities of these dyestuff ingredients, and the danger of contamination of other print colors.

I have discovered that dyestuffs and ingredients thereof which are unstable in the presence of water may be dispersed in emulsifiable non-aqueous liquids, that the resultant dispersions can be stored just as long as the dry powder without deterioration, provided the liquid has no appreciable solvent action on the dyestuff, and that the non-aqueous liquids, on the addition of water or aqueous alkalies rapidly and completely yield up the dyestuff to the water. I am thus able to prepare a readily emulsifiable base in which the colors are stable, and which can be rapidly stirred up at the print plant with water and other desired ingredients, to obtain a finished printing paste without the necessity for careful weighing of small amounts of dye powder, with the resultant errors in strength of color, and with the resultant danger of contamination of other printing pastes.

The unstable dyestuff components are largely of the class known as naphthol fast color salts, and comprise a large group of diazo compounds which can be coupled with beta-oxy-naphthoic acid and its derivatives. In general, these dyestuff components are printed onto a fabric con-

taining the base, and are coupled on the fabric. The unstable undeveloped dyestuffs are of the alkali soluble type sold under various trade names such as Rapidogen (General Dyestuff) and Dia-  
gen (du Pont); these dyestuffs are mixtures of diazo compounds and naphthols with which they can ordinarily couple, but are stabilized against reaction in aqueous alkaline solution by various agents; they are coupled on the fabric by treatments which reconstitute the two units in such form that they can couple.

The emulsifiable liquid should preferably be a solution of a film-forming substance in a volatile organic solvent, since these materials are desirable in the finished printing paste, and since they can be made sufficiently heavy in body to maintain the dyestuff dispersed through the mass. The dissolved substance should be sufficiently film-forming to be capable of forming films about the water globules, and thus ensure proper emulsification.

Provided the solution produces satisfactory water-in-oil emulsions, substantially any solvent and any film-forming substance may be used, depending on the dyestuff employed; but care must be taken that neither has any appreciable solvent action on the particular dyestuff being dispersed. The cellulose esters and ethers may be generally employed, since as a class they have solvent action on very few dyestuffs; ethyl cellulose is a preferred material because it appears to be inert to all of the water unstable dyestuffs, and because it yields good emulsions even when used in very small amounts. Milled rubber, and similar products (rubber derivative resins, chloroprene polymers, iso butylene polymers, and similar rubbery linear aliphatic polymers) and the resins derived from the polymerization of olefinic hydrocarbons are also excellent with most dyestuffs. The resins derived from aromatic hydrocarbons (cumarone-indene type) and the oxygen-containing synthetic resins (alkyd, phenolic, urea, etc.) should be used with caution, as they tend to have a solvent action on some dyestuffs. Bodied fatty oils are also satisfactory in general; and most of the natural resins may also be used. Of the common solvents, the aliphatic hydrocarbons and hydrogenated petroleum hydrocarbons likewise have no effect on the dyestuffs. The lower aromatic hydrocarbons are also satisfactory; but cuts above xylol often have a solvent action, and should be avoided. The terpenes, particularly when contaminated with oxidation products, are useful with only a limited number. The alcohols and esters should likewise be used with caution, and only after testing with the particular dyestuff.

The dyestuff may be dispersed in the liquid in any desired manner, as with a colloid mill, ball mill, three-roll mill and the like.

Typical examples of my invention are the following:

#### Example 1

|                                                    |       |    |
|----------------------------------------------------|-------|----|
| Red salt B (Schultz #155)                          | Parts | 31 |
| is dispersed in a three-roll mill in a solution of |       |    |
| 250 centipoise ethyl cellulose                     | 5     |    |
| in                                                 |       |    |
| Xylol                                              | 64    |    |

This dispersion is stable on storage; the salt in water loses color strength rapidly, particularly if not kept cool.

This dispersion can be made into an acceptable printing paste by adding—

|                                                                                                                                                                                                                   |       |   |
|-------------------------------------------------------------------------------------------------------------------------------------------------------------------------------------------------------------------|-------|---|
| Pine oil                                                                                                                                                                                                          | Parts | 3 |
| 5 Solvesso #3 (hydrogenated petroleum hydrocarbons. Boiling range 175-210° C.)                                                                                                                                    | 15    |   |
| Above dispersion and then emulsifying in                                                                                                                                                                          | 14    |   |
| 10 Water                                                                                                                                                                                                          | 68    |   |
| to yield a water-in-lacquer emulsion of excellent printing properties, which can be printed on a prepared ground (for example, one impregnated with beta-oxy-naphthoic acid anilide) to yield an excellent print. |       |   |

#### Example 2

|                                                   |       |    |
|---------------------------------------------------|-------|----|
| Fast Blue Salt B (Schultz 490)                    | Parts | 46 |
| 20 is dispersed in a colloid mill in a mixture of |       |    |
| Alkyd resin solution                              | 46    |    |
| Xylol                                             | 8     |    |

The alkyd resin solution is made by reacting 25 148 parts phthalic anhydride, 110 parts glycerol, and 125 parts castor oil fatty acids at 230° C., in the presence of carbon dioxide until the acid number is about 8, and then reducing to 50% non-volatile with a mixture of 30 parts pine oil 30 and 70 parts Solvesso #2 (hydrogenated petroleum naphtha-boiling range 135-177° C.). This dispersion, like the last, is stable on storage.

|                                 |       |     |
|---------------------------------|-------|-----|
| 35 Above dispersion             | Parts | 6.5 |
| is mixed with                   |       |     |
| Pine oil                        | 5.0   |     |
| and                             |       |     |
| Solvesso #3                     | 13.5  |     |
| 40 and                          |       |     |
| Water                           | 75.0  |     |
| is emulsified into the lacquer. |       |     |

A slight amount of acetic acid in the water phase improves the color value of this and many similar products.

#### Example 3

A duplication of Example 2, with Red Salt B (Schultz No. 155) proved unstable, apparently due to the solvent action of the alkyd resin on the salt. It should be noted that this salt is stable in ethyl cellulose.

|                                                                        |       |    |
|------------------------------------------------------------------------|-------|----|
| 55 Rapidogen Brown (General Dyestuff Corp. U. S. Patent No. 1,822,561) | Parts | 20 |
| was dispersed on a three-roll mill in                                  |       |    |
| 500 centipoise standard ethoxyethyl cellulose                          | 4     |    |
| 60 dissolved in                                                        |       |    |
| Solvesso #3                                                            | 69    |    |
| and                                                                    |       |    |
| Pine oil                                                               | 7     |    |
| This is stable on storage.                                             |       |    |

This dispersion can be made into an excellent printing paste by adding—

|                                              |      |
|----------------------------------------------|------|
| Parts                                        | 21.6 |
| Above dispersion                             |      |
| to                                           |      |
| 70 Solvesso #3                               | 14.7 |
| then emulsifying into the above              |      |
| Water, mixed with 50% caustic soda solution: |      |
| Water                                        | 61.4 |
| Caustic soda solution                        | 2.3  |

## Example 5

|                                                      |       |
|------------------------------------------------------|-------|
| Rapidogen Green B (General Dyestuff Corp.            | Parts |
| U. S. Patent No. 1,882,560) -----                    | 30    |
| is dispersed on a three-roll mill into               |       |
| 500 centipoise standard ethoxy ethyl cellulose ----- | 4     |
| dissolved in                                         |       |
| Solvesso #3 -----                                    | 59    |
| and                                                  |       |
| White pine oil -----                                 | 7     |

A printing paste can be made as in Example 4, from

|                                 |       |
|---------------------------------|-------|
| Above dispersion -----          | Parts |
| 14.3                            | 14.3  |
| Solvesso #3 -----               | 22.0  |
| Water -----                     | 61.4  |
| mixed with                      |       |
| 50% Caustic soda solution ----- | 2.3   |

## Example 6

|                                                                                  |       |
|----------------------------------------------------------------------------------|-------|
| Fast Blue Salt B (Schultz 490) -----                                             | Parts |
| is dispersed in                                                                  | 60    |
| Heavy kettle bodied linseed oil -----                                            | 30    |
| Solvesso #2 (hydrogenated petroleum hydrocarbon—boiling range 135-177° C.) ----- | 25    |
| 10                                                                               |       |

A printing paste can be made with

|                        |       |
|------------------------|-------|
| Above dispersion ----- | Parts |
| 7                      | 30    |
| Solvesso #2 -----      | 12    |
| Water -----            | 81    |

Similar results are obtained with blown oils of various sorts.

## Example 7

|                                 |       |
|---------------------------------|-------|
| The dyestuff of Example 5 ----- | Parts |
| is dispersed in a solution of   | 12    |
| 15' milled crepe rubber -----   | 23    |
| Solvesso #2 -----               | 40    |

This dispersion makes an excellent printing paste with

|                             |       |
|-----------------------------|-------|
| Above dispersion -----      | Parts |
| 30                          | 45    |
| Solvesso #2 -----           | 39    |
| 40° Bé. NaOH solution ----- | 1.5   |
| Water -----                 | 29.5  |

Other variations can be made without departing from the scope of my invention, which is defined in the claims.

This application is a continuation in part of my application Serial Number 284,210, filed July 13, 1939.

I claim:

5 1. A composition adapted to be emulsified comprising a dispersion of a material of the group consisting of dyestuffs and dyestuff components soluble in water, and dyestuffs and dyestuff components soluble in dilute aqueous alkali, in a 10 water-immiscible organic liquid having no appreciable solvent action on the dyestuff component, said liquid comprising a volatile water-immiscible organic solvent having dissolved therein sufficient of a water-insoluble film-forming substance to make the liquid capable of emulsifying water therein.

2. The composition of claim 1, in which the dyestuff is a water soluble diazo compound of the class capable of forming a dyestuff on coupling with a compound of the class consisting of beta-oxy-naphthoic acid and its derivatives.

3. The composition of claim 1, in which the dyestuff comprises an aqueous alkali soluble mixture of a diazo compound and a coupling component stabilized against reaction in aqueous alkaline solution.

4. A composition adapted to be emulsified comprising a dispersion of a material of the group consisting of diazo dyestuffs and diazo dyestuff components which are unstable on storage in aqueous solution, in a water-immiscible organic liquid in which the dyestuff is stable, said liquid comprising a volatile water-immiscible organic solvent containing sufficient of a water-insoluble film-forming substance to make the liquid capable of emulsifying water therein.

5. The method of making a textile printing paste which contains a material of the group consisting of diazo dyestuffs and diazo dyestuff components which are unstable on storage in aqueous solution, which comprises distributing the diazo dyestuff component through a water-immiscible organic liquid in which the diazo dyestuff component is stable, said liquid comprising a water-immiscible organic solvent containing sufficient of a water-insoluble film-forming substance to make the liquid capable of emulsifying water therein, and emulsifying an aqueous solvent for the diazo dyestuff component into the dispersion before use to produce a paste of printable consistency.

NORMAN S. CASSEL.